

Dec. 12, 1933.

G. REICHENBECHER ET AL

1,939,521

CENTRIFUGAL PROCESS OF LINING TUBES WITH A BITUMINOUS OR LIKE MATERIAL

Filed Jan. 13, 1932



INVENTORS.  
G. Reichenbecher And E. Grube  
BY *Mark & Clerk*  
ATTORNEYS.

## UNITED STATES PATENT OFFICE

1,939,521

CENTRIFUGAL PROCESS OF LINING TUBES  
WITH A BITUMINOUS OR LIKE MATERIAL

Georg Reichenbecher and Ernst Grube, Mulheim-Ruhr, Germany, assignors to Vereinigte Stahlwerke Aktiengesellschaft, Dusseldorf, Germany

Application January 13, 1932, Serial No. 586,450,  
and in Germany January 13, 1931

2 Claims. (Cl. 91—70)

Several processes are already known, whereby metal tubes can be lined by means of the centrifugal process with a coating of bitumen or the like or with a mixture consisting of bitumen or the like. The most widely known process consists in bringing the tube to a temperature of about 150° C. and in projecting the liquid mass into the tube by suitable rotative movement.

Another process consists in painting the inner wall of the tube with some suitable material in which bitumen is dissolved in volatile substances, and in subsequently lining by the centrifugal process the tubes with the desired mass.

The first of these processes has the disadvantage that the mass does not adhere sufficiently strongly to the wall; the second process has the disadvantage that some light, volatile constituents are left behind in the painted coating, which later on volatilize through the action of the rays of the sun and detach the centrifuged mass from the tube wall, by forming cracks.

The present invention has the object of eliminating the above disadvantages by bringing the tube to a temperature which is higher—for example, by 30° to 40°—than the working or using temperature of the bitumen to be cast. After the heating of the tube the heated casting material is very thinly applied with a brush or mop or other suitable means. Care must be taken that this coating fills even the finest pores of the tube. The tube is then allowed to cool. The warm coating mass is now applied centrifugally to the tube wall in a layer of the required thickness. Preferably the bitumen or other rust-preventing means is heated to as high a temperature as possible, so that this mass and the coating which has previously been applied in the warm

state, will key well, and gradually form a coating of the desired thickness.

In the attached drawing is shown in longitudinal section a tube of the character described. Reference numeral 10 denotes a metal tube, 11 the inside coating of the tube, preferably applied with a brush, and 12 the bituminous inner layer or lining applied warm and by centrifugal force.

What we claim and desire to secure by Letters Patent in the United States is:

1. The centrifugal process of lining tubes with a bituminous or like rust-preventing material, consisting in heating the tube to be coated from 30° C. to 40° C. above the working temperature of the rust-preventing mass to be cast, then painting the tube with a thin layer of the same rust-preventing mass, then cooling the tube, and then inserting into the tube a sufficient quantity of highly warmed lining material to form a coating of the required thickness, then rotating the tube to deposit such coating centrifugally.

2. The centrifugal process of lining tubes with a bituminous or like rust-preventing material, consisting in heating the tube to be coated from 30° C. to 40° C. above the working temperature of the rust-preventing mass to be cast, then painting the tube with a thin layer of the same rust-preventing mass, then cooling the tube, and then inserting into the tube a quantity of highly warmed lining material to form a coating, then rotating the tube and continuing the insertion of the highly warmed material until a coating of the required thickness has been deposited.

GEORG REICHENBECHER.  
ERNST GRUBE.